

Oct. 11, 1927.

1,644,692

J. B. READ ET AL

PROCESS OF ROASTING

Filed July 29, 1925



John Burns Read  
Melville F. Coolbaugh  
INVENTORS

BY

ATTORNEY

Patented Oct. 11, 1927.

1,644,692

# UNITED STATES PATENT OFFICE.

JOHN BURNS READ, OF GOLDEN, AND MELVILLE F. COOLBAUGH, OF DENVER, COLORADO, ASSIGNORS TO THE COMPLEX ORES RECOVERIES COMPANY, OF DENVER, COLORADO, A CORPORATION OF COLORADO.

## PROCESS OF ROASTING.

Application filed July 29, 1925. Serial No. 46,735.

Our invention relates to the roasting of mineral sulfides and has particularly in view a means for balancing the temperatures during the roasting operation. The invention is practised particularly in connection with a process of roasting sulfides, wherein in the air, ore and sulfur-containing gases travel concurrently or in the same direction through the furnace as disclosed in our Patent No. 1,582,347, dated April 27, 1926.

In the concurrent roasting of sulfide ores, it has been observed that it is difficult to maintain ignition in the top of the furnace, when the fuel value of the ore is low, when feeding a large tonnage, or wet, or coarse material. To maintain the ignition, it is customary to use the hot air produced by cooling the central column and rabble arms of the furnace, but in certain instances this may not be sufficient.

The object of the present invention is to take heat, in the form of gas, away from the hottest zone of the furnace and transfer such heat to the incoming charge to evaporate moisture and ignite the ore.

The difficulty of maintaining ignition is overcome in this invention by introducing the air for oxidation at a point that is lower in the furnace than that at which the ore is introduced, preferably the second or third hearth, and allowing a portion of the air, and of the gases produced, to travel upward, and the rest to travel downward. That portion which travels upward is conducted by a series of flues, either in the walls of the furnace or externally to the furnace, as shown in the drawings, and is re-admitted to the furnace, at or below the point at which the air is admitted, or it may even be turned directly into the flues. A series of dampers in conjunction with a fan, or without a fan, where flue draft is sufficient, are employed to regulate the relative proportions of air and gases which travel upward and downward.

In that section of the furnace where the gases are travelling upward, only that portion of the sulfide sulfur will be eliminated which will be necessary to keep the charge ignited; the main desulfidizing reaction will take place in that section of the furnace where the gases and solids are traveling concurrently.

By this process heat is taken from that section of the furnace which tends to be-

come too hot, and is distributed to that section which is not hot enough. The heat throughout the furnace is balanced in a way to produce more rapid and more complete oxidation of the sulfur. Ores and concentrates, which otherwise would not furnish a self-sustaining roast, can by this process, be roasted efficiently without the use of extraneous fuel.

In the drawing, the process is disclosed as being carried out in a superposed hearth furnace, although other conventional types of furnace can, with suitable modifications, be used.

Referring to the drawing for a more complete disclosure of the invention:—

The figure is a vertical section of one type of furnace suitably modified to carry out the process.

The furnace is provided with a plurality of superposed hearths 2 and a hollow vertical rotary shaft 3, having secured thereto rabble arms 4. Alternate hearths are provided respectively with central openings 5 and peripheral openings 6, through which the ore drops as it travels from hearth to hearth.

The upper end of the hollow vertical shaft 3 is connected to a flue 7, which is provided with branches 8, 9, and 10 leading into the space above the second, third, and fourth hearths and below the top hearth. The space above the top hearth is connected to a flue 11, which may be connected to a suction fan 12, the said flue 11 being provided with branch flues 13, 14, 15 and 16, leading into the spaces above the hearths which are below the first hearth.

Ore is fed in through a hopper 17 at the top of the furnace, the calcined ore being discharged through an opening 18 in the bottom of the furnace. Cold air may be admitted through the branch flue 19 and the products of combustion may be in part, or completely, led off to a stack through the branch flue 20.

Valves 21 are suitably disposed throughout the various flues for controlling the direction and amount of flow of the various gases.

## Operation.

100

Ore is fed into the upper part of the furnace through the feed hopper 17 onto the

upper hearth. The roasting process will start by drying and igniting the sulfide ore on the first hearth. The ore will continue to roast on the hearths below the first hearth, 5 and will be discharged, usually at a high temperature, through the calcine discharge 18. Cold air fed into the bottom of the hollow column 3 will be substantially raised in temperature as it enters the flue 7 on its way 10 to the branch flues 8, 9 and 10. The air entering through the flue 8 below the top hearth will in a large part pass upward together with hot gases into contact with the ore on the top hearth, providing thereby the 15 necessary heat for drying the ore and effecting ignition. The heated air passing through the branch flues 9 and 10 will furnish the necessary oxygen for combustion on the third and fourth hearths and lower hearths, 20 the gases over these hearths traveling concurrently with the ore. It may be advisable to use one, two, or three flues for the introduction of air to the furnace or any combination of flues 8, 9 and 10. In any combination 25 for introducing air a portion of it will travel upward and the remainder downward.

The direction of flow of gases on the hearths will be controlled in part by the fan 12. The fan is rotated so that the gases 30 above the top hearth will be drawn into the flue, 11, thus producing an upward current above the top hearths, whereas the fan will force the gases through the branch flues 13, 14, 15 and 16, or any of these, thus causing 35 a downward movement of gases over the ore on these hearths. The ore is stirred and moved from hearth to hearth in the customary manner by the rotating rabble arms 4.

We claim:—

40 1. A method of roasting sulfides, which comprises feeding the sulfides into and through a furnace, feeding air for oxidation into the furnace in advance of the point at which the sulfides are introduced and caus- 45 ing a portion of the hot gases to travel

counter currently to carry heat to the introduced sulfids and causing the remainder of the gases to travel concurrently with the ore.

2. A method for the concurrent roasting 50 of sulfide ores which comprises moving the ore, air for oxidation, and sulfur-containing gases in the same direction through a furnace and feeding hot gases in rear of the point at which the air for oxidation is introduced to 55 ignite the said sulfides.

3. A method for the concurrent roasting of sulfide ores, which comprises moving the ore, air for oxidation and the sulphur-containing gases in the same direction through 60 a furnace, and transferring gases from the hot zone of the furnace to the incoming charge to ignite the said ore.

4. A method for the concurrent roasting of sulfide ore, which comprises moving the 65 ore, air for oxidation and the sulfur-containing gases in the same direction through a furnace and transferring gases from the hot zone of the furnace in advance of the point 70 of entry of the incoming ore, and to the rear of the point of entry of the air for oxidation.

5. A method of roasting sulfide ores, which comprises feeding the said sulfide mineral into and through a furnace, feeding hot 75 gases countercurrently to the direction of the said ore, to ignite the said ore and eliminate such sulfide sulfur as will be necessary to keep the charge ignited and thereafter feeding air for oxidation to the said charge, 80 and moving the said air, the sulfur containing gases and the ore in the same direction through the furnace, the main desulfidizing reaction taking place in that section of the furnace, when the gases and solids are travel- 85 ling concurrently.

In testimony whereof, we affix our signatures.

JOHN BURNS READ.  
MELVILLE F. COOLBAUGH.